

## 1

3,087,812

**METALLURGICAL COMPOSITION**

Joseph H. Doss, 13417 Promenade Ave., Detroit 13, Mich.  
No Drawing. Filed May 11, 1960, Ser. No. 28,196  
1 Claim. (Cl. 75—171)

The present invention relates to new and novel high temperature heat and stress resistant nickel base alloys suitable for use at extremely elevated temperatures under substantial tensile stresses and under great pressures as in the power plant units of gas turbine engines, turbojet engines, high pressure rotors as in steam power plants and similar uses.

The art of metallurgical composition with respect to the uses cited and other similar uses involving high temperatures and great stresses has been faced in the recent past with the tendency to operate at higher and higher speeds, higher pressures and higher temperatures up to 2200° F., and above. Satisfactory service life has been obtained only with cobalt base alloys within the temperature range cited and even here the technologies have been limited by the materials available.

An object of this invention is to provide alloys suitable for use at these high temperatures and stresses, in temperatures to at least 2200° F. Another object of this invention is to provide these alloys and in addition and at one and the same time provide satisfactory, which may be equated with exceptional, resistance to oxidation, even in the presence of oxidizing atmospheres such as those obtained in the operation of jet aircraft and coal-burning gas turbines.

Another object of the invention is to provide these alloys for use at high temperatures and stresses, along with the oxidation resistance, and at the same time provide these alloys possessing a low coefficient of thermal conductivity.

Another object of the invention is to provide these alloys for use at high temperatures and stresses, resistant to oxidation, having low thermal conductivity, and also possessing freedom from temperature sink.

My experiments prove that the foregoing objects are obtained, with the provision of the highly superior properties called for, properties which possessed to the degree found in the present invention are unique, by mixing a metallurgical alloy composed of the following components, the components thereof being present in the precise proportions stated below:

| Element | Not less than, percent | Not more than, percent |
|---------|------------------------|------------------------|
| Ni      | 51.8                   | 59.4                   |
| Cr      | 5.92                   | 10.75                  |
| Co      | 12.67                  | 19.46                  |
| W       | 5.12                   | 11.2                   |
| Al      | 3.22                   | 7.2                    |
| Mo      | 3.2                    | 6.4                    |
| Nb      | —                      | 1.2                    |
| Ti      | .245                   | .687                   |
| Be      | .07                    | .19                    |
| B       | .005                   | .08                    |
| C       | —                      | 1.5                    |

<sup>1</sup> Not to exceed.

Having compounded the metal as shown above, it was tested by an independent laboratory according to procedures substantially in conformity with the general prac-

## 2

tice used by those skilled in the art of testing stainless steel and other metals for oxidation at elevated temperatures, and was found to have the following properties with respect to resistance to oxidation.

| Test temperature, ° F.: | Change in weight, gms./cm. <sup>2</sup> /hr. |
|-------------------------|----------------------------------------------|
| 1800                    | +0.00025                                     |
| 2000                    | +0.00051                                     |
| 2200                    | -0.00815                                     |

Similar tests were undertaken by the laboratory with respect to the tensile strength at elevated temperatures, substantially in conformity with the general practice used by those skilled in the art of testing stainless steel and other metals for tensile strength at elevated temperatures with the following results.

| Test temperature, ° F.: | Tensile strength, p.s.i. |
|-------------------------|--------------------------|
| 1800                    | 96,000                   |
| 1900                    | 80,000                   |
| 2000                    | 59,800                   |
| 2100                    | 38,100                   |
| 2200                    | 20,100                   |

No standard test is provided for the determination of thermal conductivity and therefore a test was devised by me for this determination, which upon calibration indicates a thermal coefficient of 6 B.T.U./hr./ft.<sup>2</sup>/° F./ft., at a metal temperature of approximately 2200° F.

Upon examination it was found that the alloy engages in thermionic electron emission to a high degree and that untreated, without the use of impregnation, oxide covering or activation, has an emission of 1 ampere per square centimeter at a temperature of 2000° F.) The above is without the addition of thorium. Experimentally, it has been found that the addition of up to 5% thorium in powdered form or master alloy to the mix during the process of mixing the alloy has no adverse effect upon the high temperature and stress properties of the alloy. In practice I believe that the addition of one-half of one percent is sufficient to benefit the emission properties of the metal by an approximate factor of 2.

## I claim:

45 A high temperature heat and stress resistant alloy containing only the following elemental substances in proportions described by percentages by weight: Nickel, 51.8% to 59.4%; chromium, 5.92% to 10.75%; cobalt, 12.67% to 19.46%; tungsten, 5.12% to 11.2%; aluminum, 3.22% to 7.2%; molybdenum, 3.2% to 6.4%; columbium, not to exceed 2%; titanium, .245% to .687%; beryllium, .07% to .19%; boron, .005% to .08%; and carbon, not to exceed .5%, provided that no component listed shall account for less or more than the listed percentage of the finished alloy.

## References Cited in the file of this patent

## UNITED STATES PATENTS

|           |               |               |
|-----------|---------------|---------------|
| 2,245,366 | Rohn et al.   | June 10, 1941 |
| 2,246,078 | Rohn et al.   | June 17, 1941 |
| 2,912,323 | Bieber        | Nov. 10, 1959 |
| 2,920,956 | Nisbet et al. | Jan. 12, 1960 |

## FOREIGN PATENTS

|              |        |               |
|--------------|--------|---------------|
| 534,855      | Canada | Dec. 25, 1956 |
| 65 1,160,309 | France | Feb. 24, 1958 |